

J. W. GEBHARD,  
ART OF HARDENING CASTINGS,  
APPLICATION FILED FEB. 12, 1915.

1,239,586.

Patented Sept. 11, 1917.

2 SHEETS—SHEET 1.

*Fig. 1.*



*Fig. 3.*



WITNESSES

R. A. Balderson  
J. M. McCorison

INVENTOR

John W. Gebhard  
by *Barclay Signs & Shoules*  
*his atty.*

J. W. GEBHARD.  
ART OF HARDENING CASTINGS.  
APPLICATION FILED FEB. 12, 1915.

1,239,586.

Patented Sept. 11, 1917.

Fig. 4.



2 SHEETS-SHEET 2.  
Fig. 5. 4a 5a



Fig. 6.



Fig. 7.



WITNESSES

R. A. Balderson  
J. T. McConville

INVENTOR

John W. Gebhard  
by *Patentee* *John W. Gebhard*  
his attorney

# UNITED STATES PATENT OFFICE.

JOHN W. GEBHARD, OF VANDERGRIFT, PENNSYLVANIA, ASSIGNOR TO UNITED ENGINEERING & FOUNDRY COMPANY, OF PITTSBURGH, PENNSYLVANIA, A CORPORATION OF PENNSYLVANIA.

## ART OF HARDENING CASTINGS.

1,239,586.

Specification of Letters Patent. Patented Sept. 11, 1917.

Application filed February 12, 1915. Serial No. 7,694.

To all whom it may concern:

Be it known that I, JOHN W. GEBHARD, a citizen of the United States, residing at Vandergrift, in the county of Westmoreland and State of Pennsylvania, have invented 5 a new and useful Improvement in the Art of Hardening Castings, of which the following is a full, clear, and exact description, reference being had to the accompanying 10 drawings, forming part of this specification, in which—

Figure 1 is a longitudinal vertical section showing a mold arranged for carrying out my process.

15 Fig. 2 is a horizontal section on the irregular line II—II of Fig. 1.

Fig. 3 is a view similar to Fig. 1 showing the casting in place after completion of the operation.

20 Fig. 4 is a sectional side elevation.

Fig. 5 is a cross section on the line V—V of Fig. 6.

25 Fig. 6 is a horizontal section, showing another casting in place, made in accordance with my invention; and

Fig. 7 is a perspective view, partly broken away, showing a vault plate casting made in accordance with my invention.

30 My invention relates to the method of making castings, particularly steel castings having a hardened face or portion formed by a layer of hardened material within the mold. The hardened material is of an exothermic character, the reaction started there- 35 in by the heat of the molten metal, giving off heat and causing a high temperature.

Heretofore in such processes two difficulties have been encountered. First, the reaction liberates gases and the hardening 40 layer must be thin in order to give the proper character of hardened portion. Hence, the hardened portion is of relatively shallow depth. Second, inasmuch as the hardening material as it melts occupies less space or 45 volume than it does before melting, it shrinks and does not entirely cover the face to be hardened.

50 My invention overcomes these difficulties and it consists broadly in feeding an additional supply of the hardening material

to the face or portion of the casting to be hardened after the melting of the hardening material begins.

In carrying out my invention, I provide 55 an additional supply of the hardening material in such relation to the face or portion to be hardened that, as the fusing of the hardening material progressively proceeds, this supply will be melted and supplied to the casting. I also arrange this additional 60 amount in such a relation that as the hardening material melts and gives out heat, thus combining with the desired portion of the casting, space will be provided to allow the slag and gases to arise, thus giving a 65 better character to the hardening portion, relieving it from sponginess, pipes, slag, etc.

I will now describe my process, referring 70 to Figs. 1 to 3 of the drawings. In these figures, 2 represents a sand-mold for casting a steel stamp-head, 3 the mold shaping cavity, 4 a sink-head cavity rising therefrom, and 5 a pouring-gate. This gate communicates through branch gates 6 with an additional sink-head cavity 7, having a gate 75 8 leading into the bottom part of the mold-shaping cavity 3. In this case I desire to harden the lower face of the steel casting and for that purpose I provide the layer 9 of the hardening compound within the mold cavity and also provide an additional column 10 of this compound within the sink-head cavity 7, this communicating with the part 8 through a connecting neck portion 11.

When steel is teemed into the gate 5, it 80 flows through the branch passages 6 and around the core-like portion 10 and the neck portion 11 of the hardening compound, and then rises over the portion 9 within the mold-forming cavity.

When the mold is filled, and when the steel begins to thicken, the reaction will begin in the hardening compound. This reaction sets free a large amount of heat and will extend progressively through the compound which melts and combines with the lower part of the steel casting, remelting this portion of the casting. As this action proceeds through the compound it will extend 85 through the neck into the portion 10, and as 90 95 100

these portions melt they will keep molten the interior of the sink-head and its neck connecting with the lower part of the mold, thus feeding an additional supply of the 5 hardening compound to the desired surface and at the same time allowing the products of the reaction, such as gas and slag, to rise through the center part of the additional sink-head.

10 When the casting is finally chilled and solid, it will be of the general form shown in Fig. 3. The slag shown at 12 resulting from the reaction of the hardening compound will lie within the sink-head below 15 its top and the hardened portion of the stamp-head will connect with the hardened portion of the sink-head which remained molten after the steel was solidified.

When the casting is removed from the 20 mold, the sink-heads are of course cut off, thus giving a stamp-head with a face hardened over its entire surface and to a depth corresponding to the depth of the hardening material supplied, the heat of reaction, etc.

25 The hardening composition employed is of exothermic nature, its reaction giving out a large amount of heat, and I may use different kinds of mixtures. For example, I have used a combination of finely ground manganese, chrome,  $\text{SiO}_2$ , aluminum and linseed oil; or a mixture of the same with nickel. One mixture which I have employed with success is manganese 44.5 parts by volume, 30 chromium 45 parts by volume,  $\text{SiO}_2$  1 part, aluminum 1 part, nickel 6 parts and oil 35 3.5 parts.

Such compositions have an exothermic reaction which starts after the steel has been poured in the mold and usually about the 40 time that the steel begins to harden.

In Figs. 4, 5 and 6 I show a mold for casting a crusher die in vertical position with the vertical angled die face hardened. In this form 2<sup>a</sup> is the mold, 3<sup>a</sup> the shaping 45 cavity; 4<sup>a</sup> sink-head and 5<sup>a</sup> the pouring gate. The pouring gate communicates with the bottom of the mold cavity through the branches 6<sup>a</sup>. The hardening composition is spread over the angular surface of the mold cavity and also extends up within the sink-head cavities.

When the molten steel is bottom cast into this mold it will fill the mold and rise within the sink-heads, and as it is beginning to 55 set, the hardening compound will begin its reaction at the bottom of the layer, this reaction proceeding upwardly, thus melting the compound and the adjacent part of the casting. During the time of reaction the 60 slag and gases will rise, and as the reaction enters the sink-head cavities, the portions of compound therein will feed down into the cavity proper to supply the required amount of material for hardening the complete face of the casting proper. When the

entire casting has finally set, the sink-head portions will contain the slag from the reaction in the cavities formerly occupied by the compound. This compound will shrink and settle more than the steel, thus leaving the 70 cavities shown.

In Fig. 7 I show a cast steel vault plate having the side softer portions 14 and the intermediate harder portion 15. In this case the hardening material is preferably 75 spread over both sides of a support such as wire netting, expanded metal or rods. This support is provided with extensions which project up within the sink-head portions of the mold cavity so that the hardening material spread thereon will extend up within these cavities. The action will be the same in this case as in the other cases, the portions of the compound within the sink-head cavities sinking down during the reaction and 80 the slag and gases rising to the top within the sink-heads.

An additional supply of the hardening reactive compound may be placed in the sink-head cavities if desired. 90

The hardening compound or alloy is proportioned so that it will not be taken up by the steel as it is poured, but will remain in solid form until the steel is poured and preferably until it begins to thicken or set. The compound must then give the exothermic reaction, raising the compound to a high melting temperature and melting the adjacent portion of the steel or metal cast. In hardening vertical faces the reaction will 95 start near the bottom of the mold and proceed rapidly upward to the top fusing the steel at the side or around the compound, the impurities rising to the top. The alloy portion of the treated section will remain liquid 100 for some time after the steel has become solid.

The hardening compound is compressed sufficiently to hold its shape, but is more or less spongy and contains air. This air will 110 supply sufficient oxygen for the initial reaction; and through the remainder of the fusing action, air will be drawn in for combustion from and through the forming mold, such as sand. 115

The hardening compound is fusible. That is, it contains fusible material so that the compound as a whole will melt and flow. It may, however, contain powdered material which has such a high melting point that it 120 may not fuse, or at least not completely fuse, but remain in solution in the fused compound. By the word "fused" or "fusible" in my claims, I intend to cover the compound whether it fuses in whole or in part. 125

The advantages of my invention will be obvious to those skilled in the art; since any desired surface or portion of the casting may be hardened throughout its entire extent, as I have overcome the difficulty in shrinking 130

of the compound layer. Furthermore a better hardened material is afforded, since the impurities are released and allowed to pass up into extensions of the casting proper 5 while the slag collects. These portions are cut off after the casting is formed. Furthermore, the hardened alloy portion of the casting is cleaned from impurities which are allowed to pass up through this alloy portion 10 while liquid.

Many variations may be made in the form and arrangement of the mold, the hardening compound and the arrangement and connections for feeding the compound into the 15 mold cavity, without departing from my invention.

I claim:

1. The method of making a casting having a hardened portion, consisting in casting 20 the metal into a mold having hardening material formed as a part thereof, and feeding an additional supply of the hardening material into the mold; substantially as described.

2. The method of making a casting having a hardened portion, consisting in casting the metal into a mold cavity containing hardening material capable of giving an exothermic reaction while fusing, and feeding additional fused hardening material to the portion of the casting to be hardened as the exothermic reaction proceeds; substantially as 30 described.

3. The method of making a casting having a hardened portion, consisting in providing 35 a mold having extensions from the shaping cavity thereof, said mold containing a hardening exothermic reactive material within the mold and its extension, and casting the metal thereinto; substantially as described.

4. The method of making a casting having a hardened portion, consisting in providing the mold with a layer of exothermic reactive 45 hardening material extending within and beyond the mold cavity proper, and causing said extension portion of the compound to feed into the mold during the reactive period; substantially as described.

5. The method of making a casting having a hardened portion, consisting in forming a 50 mold cavity with a sink-head extension open to the atmosphere, providing the mold with exothermic reactive hardening material extending into the sinkhead portion, and casting steel thereinto in contact with the hardening material in the mold cavity; substantially as described.

6. The method of making a steel casting having a hardened portion, consisting in 55 feeding the steel into a mold and bringing it in contact with a hardening material having an exothermic reaction, and feeding said material in liquid form to the portion of the casting to be hardened; substantially as described.

7. The method of making a steel casting having a hardened portion, consisting in casting steel into a mold, bringing the steel into contact with a hardening compound, having a sufficient exothermic reaction to remelt the steel portion to be hardened and the compound and thereby form a hardened alloy, and feeding the compound to the part to be hardened as the steel sets; substantially as described.

8. A mold having its molding cavity provided with an extension, said mold having a layer of exothermic reactive hardening compound extending within a part of the mold cavity and its extension, said compound being adapted to fuse under the action of the molten metal poured into the mold; substantially as described.

9. A mold having a sink-head cavity connecting with the molding cavity, the molding cavity and sink-head cavity being provided with hardening compound adapted to be contacted with and fused by the molten metal; substantially as described.

10. A mold having a molding cavity provided with an extension, and a hardening compound located within the mold and its extension, and adapted to fuse progressively when contacted with by the molten metal fed into the mold and flow to the portion of the article to be hardened, substantially as described.

11. A mold having a molding cavity provided with an extension, and a hardening compound within the mold cavity and extending into the extension, said compound being arranged to progressively fuse and give a sufficient exothermic reaction to remelt the solidified or partially solidified steel and flow to the part to be hardened to form an alloy with the steel throughout said portion; substantially as described.

12. A mold having its molding cavity provided with an extension, and a layer of hardening compound within the mold cavity and extending into the extension, the compound being adapted to start an exothermic reaction about the time when the steel begins to thicken or set, and feed sufficient of the hardening compound to alloy with the entire portion of the face to be hardened, substantially as described.

13. A mold having its molding cavity provided with a cavity extension, and a shaped layer of fusible hardening compound contained within the mold cavity and extending within the extension, the hardening compound being arranged to fuse progressively after it is contacted with by the molten metal poured into the mold and to feed as a fused compound to the surface to be hardened, said compound giving an exothermic reaction during its progressive fusing, substantially as described.

14. The method of making a casting hav-

78

75

80

85

90

95

100

105

110

115

120

125

130

ing a hardened portion, consisting in feeding the casting metal into a mold having a layer of hardening material previously applied thereto and progressively feeding 5 fused hardening material to the portion desired to be hardened to alloy therewith, substantially as described.

In testimony whereof, I have hereunto set my hand.

JOHN W. GEBHARD.

Witnesses:

W. C. LIXON,  
H. M. CORWIN.